

No. 870,364.

PATENTED NOV. 5, 1907.

A. G. HERMAN.

APPARATUS FOR HARDENING AND TEMPERING CARD TEETH.

APPLICATION FILED NOV. 9, 1906.

Fig. 1.



Fig. 3.



Fig. 2.



Witnesses.

J. P. Britt

C. C. Sippy

Inventor

A. G. Herman  
by  
O. C. Dupper

Attorneys

# UNITED STATES PATENT OFFICE.

ANTOINE GOTTFRIED HERMAN, OF AIX-LA-CHAPELLE, GERMANY.

## APPARATUS FOR HARDENING AND TEMPERING CARD-TEETH.

No. 870,364.

Specification of Letters Patent.

Patented Nov. 5, 1907.

Application filed November 9, 1906. Serial No. 342,745.

To all whom it may concern:

Be it known that I, ANTOINE GOTTFRIED HERMAN, a subject of the Emperor of Germany, residing at Aix-la-Chapelle, Germany, have invented Improved Apparatus for Hardening and Tempering Card-Teeth, of which the following is a specification.

It has heretofore been usual to harden card teeth by heating the points in a gas flame or by an electric current and then immediately and completely chilling them by a cooling liquid or by a blast of air or gas. Chilling by a cooling liquid in this manner produces points as hard as glass and consequently the points easily break off in use and in grinding down produce sparks that, especially where cotton is being worked, 15 incur the danger of fire.

With careful adjustment it is perhaps true that chilling by a blast of air or gas may produce tough and hard teeth but this can only be effected in conjunction with electrical heating as a blast of air or gas would act detrimentally upon a heating flame. Electrical heating is however much more expensive in practice than heating by a flame so that the general adoption of this method of chilling is thereby hindered.

The object of this invention is to enable card teeth 25 to be made of the desired toughness and hardness in a manner which can be readily regulated. For this purpose the heated card teeth are chilled twice and in such a way that a so-called tempering takes place after the first short preliminary chilling whereby the glass 30 hardness produced by the first chilling is somewhat lessened and the teeth after the second chilling are of a very suitable temper. The reaction that takes place is similar to that which takes place in the usual method of hardening chisels, drills and other steel tools.

According to the interval of time between the first 35 and second chilling so is the tempering weak or strong and in this way the teeth are rendered more brittle or tough as desired.

Figures 1 and 2 of the accompanying drawings are 40 sections illustrating hardening apparatus according to this invention. Fig. 3 is a partial side elevation of parts shown in Fig. 1.

In Fig. 1 the heating is effected by a gas flame and in Fig. 2 the heating is effected electrically.

The apparatus consists of a heater *a* or *a'*, preliminary chilling jets *b* or *b'*, adjustable final chilling jet *c* or *c'*, guide surface *d*, feed roller *e*, and the necessary shafts, bearings, and connecting mechanism.

In Fig. 1 the heater comprises a burner *a* fed with a 50 mixture of gas and air by a supply pipe *a*<sup>2</sup> and the mouth of which is adapted to direct the heating flame in an upward direction. The chilling jet *b* is arranged below the heater *a*, is fed with cooling medium by a pipe *b*<sup>2</sup>, and is fixed on a screw *b*<sup>3</sup> which is secured to a fixed bracket *f*. The final chilling jet *c* is arranged 55 below the jet *b* and its position in relation to the jet *b*

is adjustable for which purpose the jet *c* is fixed to a slotted plate *c*<sup>2</sup> which is fixed to the bracket *f* by means of a screw *g* the head of which bears on the plate *c*<sup>2</sup> when the screw is tightened, so as to secure the jet *c* in position after adjustment. *c*<sup>3</sup> is the cooling medium supply pipe for the jet *c*.

The guide surface *d* and a guide channel *d*<sup>1</sup> are formed in one with a bearing *h* for the feed roller spindle *e*<sup>1</sup>. The bearing *h* and bracket *f* are fixed to a common base 65 *j* so that the relative positions of the parts are maintained.

As indicated by the arrows the feed roller *e* is rotated in such direction as to bring the card teeth successively under the action of the heater *a*, jet *b* and jet *c* at a constant uniform speed.

In Fig. 2 the heater *a'* comprises a carbon electrode 70 adjustably secured to the bracket *f* by a set screw *k* and connected to one terminal of a suitable source of electricity; and a metallic plate electrode *m* connected to the other pole of the source of electricity and arranged between the card clothing and the guide *d*, a layer *n* of insulating material being interposed between the plate and guide. The other parts are arranged as in the first described arrangement.

The chilling jets *b* and *c* are so constructed that the cooling liquid emerges in a fine and completely uniform layer. Instead of cooling liquid a pasty or plastic mass, for example a mixture of water and graphite or 75 water and clay, may be employed.

The card points are heated to incandescence for a length of about one millimeter from their outer ends by the flame of the burner *a*, Fig. 1, or electrically, Fig. 2, after which they are chilled by the preliminary jet *b* or *b'* for a length of one half to three quarters of a millimeter, so that after leaving the preliminary jet the teeth still retain sufficient heat to temper the chilled piece. When the teeth points tempered to the desired degree enter the path of the final chilling jet *c* or *c'* a second and almost complete chilling takes place, 90 the teeth retaining only sufficient heat to vaporize the adhering particles of liquid.

As the distance between the final chilling jet and the preliminary chilling jet is increased the greater is the tempering down of the card points and the softer yet 95 tougher they become. The degree of hardness or temper of the card teeth may therefore be easily regulated as desired by adjusting the distance between the two chilling jets.

What I claim is:

1. Apparatus for hardening and tempering card teeth comprising a heater, a preliminary cooling device, and a final cooling device, substantially as set forth.
2. Apparatus for hardening and tempering card teeth comprising a heater, a preliminary cooling device, and a final cooling device adjustable relatively to said preliminary cooling device substantially as set forth.
3. Apparatus for hardening and tempering card teeth,

- comprising a heater, a preliminary cooling device, a final cooling device and means for successively conveying card teeth under the influence of said heater, said preliminary cooling device and said final cooling device, substantially as set forth. 45
4. Apparatus for hardening and tempering card teeth comprising a heater, a preliminary cooling device, a final cooling device, adjustable relatively to said preliminary cooling device, and means for successively conveying card teeth under the influence of said heater, said preliminary cooling device and said final cooling device, substantially as set forth. 50
5. Apparatus for hardening and tempering card teeth comprising means for heating the points of card teeth, a device arranged near to said heating means adapted to chill the heated card teeth, a second cooling device, and means for successively conveying card teeth under the influence of said heating means, said first cooling device and said second cooling device, substantially as set forth. 55
6. Apparatus for hardening and tempering card teeth comprising means for heating the points of card teeth, a device arranged near to said heating means adapted to chill the heated card teeth, a second cooling device adjustable relatively to said first cooling device, and means for successively conveying card teeth under the influence of said heating means, said first cooling device and said second cooling device, substantially as set forth. 60
7. Apparatus for hardening and tempering card teeth comprising means for heating the points of card teeth, a nozzle arranged near said heating means adapted to deliver a jet of cooling medium onto the heated card teeth, a second similar cooling nozzle adjustable towards and away from said first cooling nozzle, and means for successively conveying card teeth under the influence of said heating means, the cooling jet from said first nozzle and the cooling jet from said second nozzle, substantially as set forth. 65
8. Apparatus for hardening and tempering card teeth comprising a gas burner the flame of which is adapted to heat card teeth, a preliminary cooling device, a final cooling device adjustable relatively to said preliminary cooling
- device and means for successively conveying card teeth under the influence of said heater, said preliminary cooling device and said final cooling device, substantially as set forth. 70
9. Apparatus for hardening and tempering card teeth comprising a gas burner the flame of which is adapted to heat card teeth, a nozzle arranged near said burner, adapted to deliver a jet of cooling medium onto the heated card teeth, a second similar cooling nozzle adjustable towards and away from said first cooling nozzle and means for successively conveying card teeth under the influence of a flame from said burner, the cooling jet from said first nozzle and the cooling jet from said second nozzle, substantially as set forth. 75
10. Apparatus for hardening and tempering card teeth comprising a guide over which card clothing may be passed, means facing said guide adapted to heat the teeth of card clothing on said guide, a device arranged near to said heating means adapted to chill the heated card teeth, a second cooling device adjustable relatively to said cooling device and means for drawing card clothing over said guide to bring the card teeth successively under the influence of said heating means, said first cooling device and said second cooling device, substantially as set forth. 80
11. Apparatus for hardening and tempering card teeth comprising means for heating the outer end portions of card teeth, a preliminary chilling device arranged near to said heating means adapted to chill the outer end portions of the heated card teeth for a length less than that heated by said heating means, and a second device adapted to completely chill the heated and partly chilled card teeth adjustable relatively to said preliminary chilling device, substantially as set forth. 85

Signed at Aix-la-Chapelle, Germany this 18th day of October 1906.

ANTOINE GOTTFRIED HERMAN.

Witnesses:

HENRY QUADFLIEG,  
ELIESE KALBUSCH.